

## UNITED STATES PATENT OFFICE.

OSCAR V. MAURER, OF EAST CLEVELAND, OHIO.

## INCANDESCENT LAMP.

No Drawing.

Application filed July 17, 1925. Serial No. 44,364.

This invention relates to incandescent electric lamps and has for its object the provision of a new and improved filamentary material possessing special physical and electrical properties. Of metallic filamentary materials tungsten is the only substance which has heretofore received extended commercial use and this despite certain practical disadvantages, chief among which are a decided tendency towards crystallization accompanied by what is known as "off setting," namely a displacement of the crystals relative to each other resulting in weakening or breakage of the metallic strand; and a rather low specific resistance, although the latter is coupled with a rather high temperature coefficient which holds the current consumption at a proper point during actual use, but results in an overstrong rush of current the instant a lamp is turned on, which frequently produces rupture of the filament at this instant. It is very difficult to reduce tungsten to the form of a ductile wire (see Coolidge Patent No. 1,082,933, issued December 30, 1913), and apparently this difficulty becomes so enhanced by the inclusion of even small proportions of other elements as to render it difficult if not impossible to remedy these difficulties by the addition of other metallic ingredients in small quantities.

Tantalum has also been suggested and patented (see Von Bolton Patent No. 817,732, issued April 10, 1906) as a filamentary material, and exhibits certain features decidedly superior to tungsten, notably a specific electric resistance double that of tungsten at room temperatures combined with a temperature coefficient only two-thirds that of tungsten. Accordingly at the working temperature a tantalum filament will be substantially larger than a tungsten filament of the same length and capacity, which affords increased light emitting surface combined with a smaller tendency to draw an unduly great initial current. Tantalum, however, has exhibited certain practical defects, notably: a tendency to disintegration under the influence of alternating current; a tendency, in the presence of any residual nitrogen to become brittle with use, especially at the comparatively cool places where the filament is attached to the leading-in wires; and a tendency for the strongly heated portions to

become so thoroughly annealed after a short use as to sag by their own weight or to become seriously stretched and deformed as a result of mechanical shocks.

I have discovered that tantalum is able to assimilate a substantial proportion of metallic tungsten with the production of an alloy having advantageous physical and electrical properties for the purpose in view. For use as a drawn wire I prefer an alloy containing about 90% of tantalum and 10% of tungsten, although advantageous results are secured by the use of a considerably smaller proportion of tungsten or by a larger proportion up to the limit of what can be drawn into wire conveniently in case the proportion of tungsten be greater than about 20%.

At percentages above those which can be reduced to filament form by drawing in dies it is possible to work the alloy by rolling into strips and shearing into ribbons. The addition of tungsten within the limits herein described serves to enhance the electrical resistance, decrease the resistance temperature coefficient, decrease the tendency to embrittlement by chemical reaction with residual gases, and afford greater rigidity during and after heating. Apparently the melting point of the alloy is slightly greater, or at least not less than, that of pure tantalum. The light produced is of a very satisfactory color and the filaments exhibit no objectionable tendency towards crystallization or off-setting. The maximum electrical resistance is produced when the two metals are present in equal proportions which for some purposes is the most desirable composition.

It is well known that the specific electric resistance of tungsten when cold is comparatively low, being less than that of tin, platinum, iron, nickel, and even than brass which is supposed to be a metal of comparatively high conductivity. On the other hand the resistance temperature coefficient is rather high which two properties together require lamp filaments made from pure tungsten to have a sufficiently large cross section to carry the necessary current under operating conditions and this entails the filament of such low resistance when cold that a decided over rush of current is produced. Alloying with tantalum increases the specific electric resistance when cold and decreases

the temperature coefficient thereby overcom-  
ing this tendency.

On the other hand tantalum alone offers  
the disadvantages of being unduly soft and  
5 jarred out of shape by shocks. By alloying  
the two metals together it is possible to pro-  
duce an incandescent body having a melt-  
ing point at least about 2800° centigrade  
and a specific electrical resistance more than  
10 twice that of tungsten combined with a re-  
sistance temperature coefficient less even than  
that of tantalum. I am not aware of any  
other combination of metals which will pro-  
duce this result, although there are at least  
15 two alloys of tungsten and tantalum which  
will do this, namely those having a prepon-  
derance of tungsten and those having a pre-  
ponderance of tantalum and I desire to  
claim and secure both compositions although  
20 I preferably employ that composition having  
a preponderance of tantalum and have  
directed my specific claims to this end.  
I do not exclude the use of minor propor-  
tions of other ingredients designed for the  
25 purpose of facilitating radiation or emission  
of light waves, electrons, etc., such as tho-  
rium, zirconium, and other rare-earth metals,  
or such non-metallic additions as rare-earths  
themselves or the alkaline earth oxides  
30 which, if used at all, occur only in small  
amounts and produce only their own par-  
ticular effect.

Having thus described my invention what  
I claim is:

1. An incandescent body for electric lamps 35  
consisting of an alloy containing from 50%  
to 99% metallic tantalum and 1% to 50%  
of metallic tungsten combined together in the  
form of a homogeneous alloy.
2. An incandescent body for electric lamps 40  
consisting of a wrought strand of a binary  
alloy of tantalum and tungsten wherein the  
tantalum constitutes at least about 50% of  
the whole and the tungsten at least about  
10%.
3. An incandescent body for electric lamps 45  
consisting of a solid solution alloy contain-  
ing at least about 80% of tantalum and at  
least about 1% of metallic tungsten.
4. An incandescent body for electric lamps 50  
consisting of a drawn wire of an alloy con-  
taining tantalum and tungsten wherein the  
tantalum comprises about 90% of the whole.
5. A metallic incandescent body for elec-  
tric lamps consisting of an alloy containing 55  
essentially tantalum and tungsten having a  
melting point at least about 2800° centigrade  
and a specific electrical resistance when cold  
more than twice that of tungsten combined  
with a resistance temperature coefficient less 60  
than that of tantalum.

In testimony whereof I hereunto affix my  
signature:

OSCAR V. MAURER.